

# UNITED STATES PATENT OFFICE.

HENRY W. PARTIN, OF PORTSMOUTH, VIRGINIA.

## METHOD OF HARDENING AND TOUGHENING METAL.

937,263.

Specification of Letters Patent.

Patented Oct. 19, 1909.

No Drawing.

Application filed September 10, 1908. Serial No. 452,479.

*To all whom it may concern:*

Be it known that I, HENRY W. PARTIN, a citizen of the United States, residing at Portsmouth, in the county of Norfolk and 5 State of Virginia, have invented certain new and useful Improvements in Methods of Hardening and Toughening Metal, of which the following is a specification.

My invention relates to an improvement 10 in a method for hardening and toughening tools of iron or steel used for any class of work such, for instance, as cutting or punching.

The object of the invention is to harden 15 and toughen tools by subjecting them to a certain process which will be hereinafter described, making the tool much harder and tougher than tools now used, thus permitting them to be used for many purposes for 20 which the ordinary tool could not be used, and in performing these functions the tools are in no wise injured for further use.

A further object of the invention is to harden and toughen any kind of metal, such 25 as armor plate, iron or steel rails, and other similar articles of manufacture.

The tool or metal previous to its treatment 30 is brought to the proper heat, which is different with different articles, some articles requiring greater heat than others. The metal or tool while in this heated condition is rolled or dipped into a compound consisting of pulverized borax, bicarbonate of soda, common salt, and salts of cobalt mixed in 35 equal proportions. The metal when in its heated condition will absorb the compound or powder as the heat opens up the pores, so that the compound passes entirely through the metal, and the metal becomes toughened.

40 I am enabled to use only borax and bicarbonate of soda to obtain results, but prefer to combine the borax and soda with common salt, omitting the cobalt or including both salt and cobalt with the soda and borax.

45 After the heated metal has been dipped, rolled, or has received the powder or compound thereupon in any approved manner it is then immersed in a solution consisting of the following ingredients: fifty gallons of 50 water; one-half pound of lime, either shell or rock lime; one ounce of sal ammoniac; one ounce of bicarbonate of soda; one ounce of

borax, and one ounce of sweet spirits of niter or linseed oil may be used alone as a bath instead of using the above named bath.

55 In immersing the heated metal after the compound or powder has been placed thereupon into the solution above given, the tool or metal is hardened as in the ordinary tempering process, but by subjecting it to this 60 solution composed of the ingredients named the metal or tool becomes very hard so that when the article has received the treatment it is a much tougher and harder article.

In hardening tools the tool may receive 65 the treatment after it has been fashioned into its proper shape or the metal may be treated before it is shaped or fashioned and then the tool fashioned into its proper shape.

From the foregoing it will be seen that I 70 have provided means whereby metal and tools made of either steel or iron can be hardened and toughened without producing undue brittleness, and when applied to the tempering solution after having received the 75 compound upon the heated article it is hardened and toughened, creating a tool superior and more durable than any now on the market.

Having fully described my invention, 80 what I claim as new and desire to secure by Letters Patent is:

1. The herein-described method of treating iron or steel consisting in treating the heated metal to a powder compound containing 85 borax and soda and then tempering the metal.

2. A method for treating iron or steel consisting of treating the heated metal to a powder compound containing borax, soda, 90 and common salt and then subjecting the metal to the tempering process.

3. A method for treating iron or steel consisting of treating the heated metal to a compound containing borax, soda, cobalt and 95 common salt and then subjecting the metal to the tempering process.

4. A method for treating iron or steel consisting in treating the heated article to a compound containing borax and soda and 100 then inserting the metal in a bath containing water, lime, soda, and borax.

5. A method for treating iron or steel consisting in treating the heated article to a

compound containing borax and soda, and then inserting the metal in a bath containing water, lime, sal ammoniac, soda, and borax.

6. A method for treating iron or steel consisting in treating the heated article to a compound containing borax and soda, and then inserting the metal in a bath containing water, lime, soda, borax, and sweet spirits of niter.

10 7. A method for treating iron or steel consisting in treating the heated metal to a

compound containing borax, soda, salt, and cobalt, and then inserting the metal in a bath containing water, lime, sal ammoniac, soda, borax, and sweet spirits of niter.

15

In testimony whereof I affix my signature, in the presence of two witnesses.

HENRY W. PARTIN.

Witnesses:

HERBERT C. EMERY,  
VERNON E. HODGES.